

# UNITED STATES PATENT OFFICE.

RUDOLF WEEBER, OF BÄRN, AUSTRIA.

## MANUFACTURE OF VARNISH.

1,257,562.

Specification of Letters Patent. Patented Feb. 26, 1918.

No Drawing.

Application filed February 19, 1914. Serial No. 819,756.

To all whom it may concern:

Be it known that I, RUDOLF WEEBER, engineer and factory manager, a subject of the Emperor of Austria, residing at Bärn, 5 Moravia, in the Empire of Austria, and whose post-office address is Bärn, Moravia, Empire of Austria, have invented a certain new and useful Improved Manufacture of Varnish, of which the following is a specification.

This invention relates to the manufacture of a varnish from semi-drying oils, more particularly train oils, which varnish serves the purpose of the covering varnish made 15 from linseed oil, and therefore can be used for the manufacture of oil cloth and linoleum.

To that end, it has been suggested to treat oils by heating them in a vacuum, or with 20 superheated steam or inert or neutral gases, in order to remove injurious ingredients. Such processes have the drawback however that they do not remove completely all the free fatty acids, as in these circumstances 25 the latter undergo further decomposition and conversion. In any case, these processes either considerably reduce the yield of varnish, or yield an inferior badly drying varnish.

30 A process is known in the manufacture of varnish from linseed oil, in which a small quantity of alkalis, carbonates of alkalis or alkaline earths (more particularly lime) are added to heated fatty oils. These addi-

35 tions are admissible only in a maximum quantity of  $\frac{1}{2}\%$  of the quantity of oil, as a larger addition stops polymerization and completely does away with the drying quality of the varnish obtained. For that

40 reason the admissible quantity in the known process is given as  $\frac{1}{2}\%$ .

Semi-drying oils, such as train oils, contain however from 15-20% and frequently even 30% of free fatty acids. If semi-drying 45 oils, more particularly train oils, were treated by the process suggested for fatty oils, and the necessary quantity of alkalis added to the train oils during the process of boiling, polymerization would be prevented, and the drying or siccative property 50 of the varnish obtained, would be destroyed; as the soaps, lime or alkaline soaps formed counteract the said properties. The addition of larger quantities of alkalis during 55 the boiling process would moreover bring

about an extensive saponification and hydrolysis of the train oils.

The said drawbacks are obviated by the process according to this invention as regards oil cloth and linoleum manufacture. 60 This is attained by the fact that the free fatty acids which are saponified by the addition of a lye are separated from the oil before the boiling process, so that only pure oil is boiled. The oils are first treated in a 65 cold or moderately heated state with soda or lime or lye of suitable concentration, whereupon the soap thus formed is allowed to settle from the free fatty acids and alkali hydrate, and is decanted or separated in 70 some other way from the pure oil. The said pure oil consisting only of the fatty acids originally combined, and separated above the soap, is then submitted to a boiling process as for varnish manufacture, 75 preferably at the same time being polymerized in the known manner or boiled with or without siccatives. Before the boiling, any traces of suspended alkali particles which cannot be completely removed from the oil, 80 can be neutralized by a little acid.

The above process is intended for all kinds of train-oil, (fish-oil) that are of a glyceridic character, as well as for such that chiefly consist of compound ethers of or 85 containing monohydric alcohols, the glycerids being hydrolyzed in the process through the combination of bases and the hydrolyzed acids subsequently treated.

As an example of the execution of the 90 process the following is given:

Dark-brown train-oil or fish oil, is primarily mixed with soda-lye and agitated, and the mixture is left undisturbed for two days at an approximate temperature of 65° 95 C. until the produced soap has settled at the bottom. The pure oil that collects at the top is skimmed out, and is, for example, boiled down for seven hours at a temperature of 300° C. with a siccative cobalt. A 100 part of the thus obtained mass is set upon a wax-layer or foundation, and dries in about seven hours upon being subjected to a temperature of 75° C.

Having now particularly described and 105 ascertained the nature of my said invention and in what manner the same is to be performed, I declare that what I claim is:

1. The process for the manufacture of varnish from semi-drying oils, such as train- 110

oil, which consists in treating the oil with a lye in a comparatively cold state to saponify the free fatty acid, separating the soap thus formed from the oil, and polymerizing the oil until varnish is produced.

2. The process for the manufacture of varnish from semi-drying oils, such as train-oil, which consists in treating the oil with a lye to saponify the free fatty acid, removing particles of excess lye suspended in the oil, separating the soap from the oil, and polymerizing the oil until varnish is produced.

3. The process for the manufacture of

varnish from semi-drying oils, such as train-oil, which consists in treating the oil with a lye to saponify the free fatty acid, separating the soap thus formed from the oil, and polymerizing the oil with siecatives until varnish is produced.

In testimony whereof I have signed my name to the foregoing specification in the presence of two subscribing witnesses.

RUDOLF WEEBER.

Witnesses:

AUGUST FUGGER,  
GUSTAV WOLFE.